# EUROPEAN PATENT SPECIFICATION

(11) **EP 1 171 492 B1**
(45) Date of publication and mention of the grant of the patent: **03.09.2003**
(21) Application number: 99967997.0
(22) Date of filing: 22.12.1999
(51) Int. Cl.: C08F 230/02, C08F 228/02, C08F 8/40, D21H 17/34

(54) **BIFUNCTIONAL POLYMERS**
BIFUNKTIONELLE POLYMERE
POLYMERES BIFONCTIONNELS

(30) Priority: 06.04.1999 US 286742; 06.04.1999 US 286745
(43) Date of publication of application: 16.01.2002
(73) Proprietor: MINERALS TECHNOLOGIES INC., New York, New York 10174 (US)
(72) Inventor: DRUMMOND, Donald, Kendall, Quakertown, PA 18951 (US); WERNETT, Patrick, Clinton, Upper Black Eddy, PA 18972 (US)
(74) Representative: Bawden, Peter Charles
(86) International application number: IB9902101
(87) International publication number: WO00059965

(56) References cited:
- EP-A- 0 112 520
- EP-A- 0 113 438
- EP-A- 0 643 081
- WO-A-98/06898
- DE-A- 4 343 993
- DE-A- 19 508 936
- US-A- 3 926 718
- US-A- 5 336 316
- DATABASE WPI Section Ch, Week 9631 Derwent Publications Ltd., London, GB; Class A14, AN 1996-307216 XP002138961 & JP 08 134792 A (NIPPON PMC KK), 28 May 1996 (1996-05-28)

## Description

The present invention relates to paper containing polymer compositions which contain sulfonate and/or phosphonate groups particularly as retention or strength aids, and to paper making methods, involving such polymer compositions.

### BACKGROUND OF THE INVENTION

Currently, filler levels in paper are limited, in part, by paper strength losses as filler levels increase. Minimum strength requirements prohibit the paper maker from adding more filler which is desirable because fillers are generally less expensive than the wood fiber that they replace. The ability to add more filler would allow the paper maker to reduce paper production costs by replacing the more expensive fiber. In order to achieve higher filler levels, the paper maker needs fillers, additives or processes which increase paper strength. Historically, the paper maker has used filler modification, wet end additives and fiber modifications to achieve higher strength levels in paper. Filler modifications have included changing filler type, changing filler particle size and surface treatments of fillers. Wet end additives have included synthetic and natural polymers such as polyacrylamides and starches. Fiber modifications have included changing fiber type and fiber processing.

In general, the paper industry is trending toward higher filler levels to reduce costs and as a result is continually looking for ways to improve paper strength. To achieve this, a new generation of strength aids is required for the paper industry.

### PRIOR RELATED ART

In U.S. Patent No. 3,709,780, there is disclosed paper products having improved strength properties by adding to the cellulose paper dispersion a chitin-based compound of a graft copolymer of 2-acrylamide-2-methylpropanesulfonic add (AMPS) onto a chitosan substrate.

In U.S. Patent No. 3,692,673, there is disclosed polymers of acrylamido sulfonic acids, and their salts, which are useful as flocculants for aqueous systems.

In U.S. Patent No. 4,555,558, there is disclosed water soluble terpolymers of AMPS; N,N-dimethylacrylamide; and acrylonitrile. These terpolymers are reported to provide high temperature fluid loss additives and rheology stabilizers for high calcium-containing brine clay drilling fluids.

In U.S. Patent No. 3,926,718, there is disclosed the use of water-soluble block polymers having blocks derived from a water-soluble monomer and blocks derived from N-vinyl pyrrolidone. These polymers are reported to perform as drainage and retention aids for paper webs where the polymer is added to a pulp slurry.

In U.S. Patent No. 5,075,401, there is disclosed a graft copolymer made by a free radical reaction mechanism. The copolymer uses polymeric units of acrylamide, acrylic acid and/or AMPS.

### SUMMARY OF THE INVENTION

An object of the present invention is to provide a polymer having varied substituent groups having varied functions or utilities. One specific objective is to provide a polymer useful for binding mineral fillers, particularly to polysaccharide materials, such as paper pulps and the like. Such and other objectives are achieved in that the present invention provides the use of polymers having phosphonated and sulphonated substituent groups in paper making such that the polymer is multifunctional in its use. Optional amide substituents are used to reduce electrostatic charge density or for increasing hydrogen bonding. An advantage of the polymer is the flexibility of using it for multiple purposes. Other advantages will be discerned by those skilled in the art in familiarizing themselves with this specification.

### DETAILED DESCRIPTION OF THE INVENTION

One embodiment of the present invention is the use in paper making of a polymer composition having a polymeric core, one or more phosphonated substituents effective for bonding with an inorganic material, and one or more sulphonated substituents effective for bonding with a polysaccharide material.

Preferably, the polymeric core comprises one or more polymer units selected from polymerizable monomeric units, such as by condensation or free radical methods, preferably from allylic units, epoxidic units, and vinylic units. The polymeric core can be composed of varying proportions or sequences of substituted or unsubstituted monomeric (or polymeric units of allylic units, epoxidic units and vinylic units. Not all allylic unit, epoxidic units, or vinylic units need be the same as the other respective allylic units, epoxidic units, or vinylic units, but they can be. Such difference can result from hydrolysis reactions, among others, and whether intended or not. Such allylic, epoxidic and vinylic units can have one or more of the phosphonated or sulphonated substituents attached before or after polymerization. Such units of the core can be repeating in a predictable sequence or repeat randomly.

An allylic unit can be one derived from a compound with the moiety of CH₃CH₂ = CH-. A preferred allylic unit is a polyacrylamide unit. The epoxidic unit can be one derived from a compound with the moiety of

The vinylic unit can be derived from a compound with the moiety of CH₂ = CH-. A preferred vinylic unit is vinylphosphonate. Any one or more of the hydrogen atoms may be substituted before, during or after polymerization. The proportions of allylic units, epoxidic units, and vinylic units can vary widely, or a polymer can be composed of only one type of unit alone or various combinations thereof. Whether a polymer is made of only allylic units, only epoxidic units, only vinylic units or a combination of these types of units, the units of each type may be the same or different because of substitution. In a more preferred embodiment, the amount or proportion of the polyacrylamide units or the epoxidic units to the balance of the polymer composition is effective for reducing the electrostatic charge density of the polymer composition or for increasing the hydrogen bonding to the polysaccharide material or, more preferably, both.

Polysaccharide materials include cellulose, starch and other similar natural and synthetic glycosidic-linked saccharides. Preferred polysaccharides are cellulose, more preferably wood fiber and bagasse; even more preferably, cellulosic fibers for paper production.

In one embodiment, the present invention provides the use of a polymer composition comprising a various mixture of linking monomeric units, amide or epoxide monomeric units, phosphonated monomeric units and sulphonated monomeric units.

The preferred linking monomeric unit can be represented by the formula - CH-CH(R₁)-, wherein R₁ is hydrogen, a halogen or a lower alkyl.

The cationic or neutrally charged amide monomeric unit can be represented by the formula: wherein "C" is carbon; "O" is oxygen; "N" is nitrogen; "A" is an unsubstituted or substituted (C₁-C₆) alkylene or a hydrogen, wherein the substituents are independently selected from (C₁-C₃) alkyls and halogens, "B" is hydrogen, hydroxyl, or ether; preferably hydrogen. The nitrogen, N, can also be a quaternary nitrogen, including, but not limited to, combinations of the groups above; and "R₁" and "R₂" are each independently hydrogen, halogen or a (C₁-C₃) alkyl. "A", if not hydrogen, is an (C₁-C₆) alkylene, e.g., methylene, ethylene, propylene, butylene, pentylene or hexylene. Such alkylenes can have a (C₁-C₃) alkyl substituent, e.g., methyl, ethyl or propyl. The halogen which can be a substituent on an alkyl or alkylene chain herein is selected from bromine, chlorine and fluorine atoms. For R₁ and R₂, the (C₁-C₃) alkyls are methyl, ethyl and n-propyl.

The preferred epoxide monomeric unit can be represented by the formula -CHR-O-CH₂, wherein R is hydrogen or lower alkyl or alkylene, e.g. alkylene having one to six carbon atoms.

The preferred phosphonated monomeric unit can be represented by the formula wherein "P" is phosphorus; "O" is oxygen; and "A" is selected from an unsubstituted or substituted (C₀-C₅) alkylene, wherein the substituent is independently selected from (C₁-C₃) alkyls and halogens, or from carbonyl (-CO-), carbonylaminos (-CO-NE-, where "E" hydrogen, hydroxyl, or ether), alkylenecarbonylaminos (e.g. -(CH₂)ₓ -CO-NE-, where x is an integer), carbonylaminoalkylenes (e.g. -CO-NE-(CH₂)ₓ -), or alkylenecarbonylamino-alkylenes (e.g. -(CH₂)ₓ - CO- NE- (CH₂)ₓ -); and "D" is a hydrogen proton or a salt moiety selected from aluminum, calcium, iron, lithium, magnesium, potassium, sodium, titanium and zinc ions. When in a salt moiety, the substituents are such that results in an electronic balance for the substituent group. The "A" is an (C₀-C₅) alkylene, e.g., nothing, methylene, ethylene, propylene, butylene, pentylene or, hexylene. However, such preferred alkylenes can have one or more (C₁-C₃) alkyl substituent(s), e.g.. methyl, ethyl, or propyl. The halogen which can be a substituent on an alkyl chain herein is selected from bromine, chlorine, and fluorine atoms. Such halogens can be substituents on the alkylene chain also. When "A" is represented as -C(=O) - N(-E) - then E is hydrogen, hydroxyl, or ether; preferably hydrogen. The nitrogen, N, can also be a quaternary nitrogen, including, but not limited to, combinations of the groups above.

When "D" is a hydrogen proton, - PO₃ - D can be represented as -P(=O)(-OH)(-OH). When "D" is a salt moiety, then -PO₃ - D can be shown by examples as
-(PO₃)⁻² (Na⁺¹)₂ when sodium is the moiety; or
-(PO₃)⁻² (Ca⁺²)₁ when calcium is the moiety.
"D" may also represent a pairing of hydrogen and salt moiety. e.g. -(PO₃) H⁺¹ Na⁺¹.

The invention is paticular concerned with filled paper and the filler is preferably an inorganic material. Although such is contemplated in the present invention, the invention is not necessarily limited to such inorganic materials. In some preferred embodiments, the inorganic material is a filler or other additive for paper compositions. A preferred inorganic material is one derived from or made with calcium containing matter, such as some clays or natural calcium carbonate. Another preferred inorganic material is precipitated calcium carbonate.

The preferred sulphonated monomeric unit can be represented by the formula wherein "S" is sulfur, "O" is oxygen; and "A" is selected from an unsubstituted or substituted (C₀-C₆) alkylene, wherein the substituent is independently selected from (C₁-C₃) alkyls and halogens, or from a carbonyl (-CO-), carbonylaminos (-CO-NE-, where "E" hydrogen, hydroxyl, or ether), alkylenecarbonylaminos (e.g. -(CH₂)ₓ -CO-NE-, where x is an integer), carbonylaminoalkylenes (e.g. -CO-NE-(CH₂)ₓ -), or alkylenecarbonylaminoalkylenes (e.g. -(CH₂)ₓ - CO- NE- (CH₂)ₓ -); and "D" is a hydrogen proton or a salt moiety selected from aluminum, calcium, iron, lithium, magnesium, potassium, sodium, titanium and zinc ions. When in a salt moiety, the substituents are such that results in an electronic balance for the substituent group. The "A" is an (C₀-C₅) alkylene, e.g., nothing, methylene, ethylene, propylene, butylene, pentylene or, hexylene. However, such alkylenes can have a (C₁-C₃) alkyl substituent, e.g., methyl, ethyl, or propyl. The halogen which can be a substituent on an alkyl chain herein is selected from bromine, chlorine, and fluorine atoms. Such halogens can be substituents on the alkylene chain also. When ''A" is represented as - C(=O) - N(-E) - then E is hydrogen, hydroxyl, or ether; preferably hydrogen. The nitrogen, N, can also be a quaternary nitrogen, including, but not limited to, combinations of the groups above. For example, when D is sodium, - SO₃ - D can be represented as - SO₃⁻Na⁺. When D is an alkyl group, - SO₃ - D can be represented as - SO₃CH₃.

Non-limiting examples of the substituent groups are:
I. Phosphonate Substituents
   - PO₃H₂ - PO₃(CH₃)₂ - PO₃(H)(CH₃)
   - CH₂PO₃H₂ - CH₂PO₃(CH₃)₂ -CH₂PO₃(H)(CH₃)
   - C(=O) NH CH₂ PO₃H₂
II. Sulphonate Substituents
   -C(=O) NH CH₂ SO₃ H -C(=O) NH C(CH₃)₂CH₂ SO₃ H
   -CH₂C(=O)NH C(CH₃)₂CH₂SO₃ H - CH₂C(=O)N(CH₃)C(CH₃)₂CH₂SO₃H
III. Cationic or Neutrally Charged Amide Substituents
   -C(=O)NH₂ - CH₂C(=O)NH₂
   -C(=O)NH CH₃ - C (=O)N⁺(CH₃)₃

Preferably, the molecular weight of the composition having the above core and substituents ranges from about 100,000 to about 20,000,000. When produced without the optional cationic or neutrally charged amide substituent, the more preferred molecular weight ranges from about 500,000 to about 5,000,000. When produced with the optional cationic or neutrally charged amide substituent, the more preferred molecular weight is about 500,000 to about 5,000,000.

The compositions used in the present invention can be produced with varying proportions or ratios of the molar units of the phosphonated substituents, the sulfonated substituents, and the optional cationic or neutrally charged amide substituents. The molar unit ratio of phosphonated substituents to sulfonated substituents can range from about 99/1 to about 1/99, but is preferably from about 45/55 to about 1/99, more preferably from about 10/90 to about 1/99. When the optional cationic or neutrally charged amide substituents are present in the produced polymer, such substituents are preferably predominate in proportion to the other substituents, preferably in a ratio of about 1/1, more preferable about 10/1 or higher relative to the phosphonated substituent. The ratio of the other two substituents to each other can remain as stated hereinabove. Accordingly, a preferred molar unit ratio of (cationic or neutrally charged amide substituents) to (sulphonated substituents) to (phosphonated units) is (from about 70 [preferably about 85] to about 90) molar units of cationic or neutrally charged amide substituents to (from about 0 [preferably about 10] to about 30) molar units of sulphonated substituents to (from about 0 [preferably about 5] to about 10) molar units phosphonated units. For examples, molar unit ratios of cationic or neutrally charged amide substituents/sulphonated units/phosphonated units of 85/10/5, 89/10/1 and 90/9/1. Other exact ratios are also preferred when in the stated ranges. While the sequencing of the units may vary according to the intended use, there is no general requirement or preference and the invention is not to be limited to any particular sequence illustrated herein. Additionally, the terminal units of the polymer , as well as other units and substituents, can be other than the units or substituents described as long as the presence of such does not interfere with the benefits of the present invention. Similarly, some degree of cross-linking may occur, but preferably is substantially absent.

In one preferred embodiment of the present invention the phosphonated substituent can be described as having the chemical structure of - PO₃H; the sulphonated substituent as having the chemical structure of -C(O)NHC(CH₃)₂CH₂SO₃H; and the cationic or neutrally charged amide substituent as having the chemical structure of -C(O)NH₂. Such polymer can be synthesized by the polymerization of varying proportions of vinylphosphonic acid monomers; 2 -acrylamido- 2 -methylpropanesulfonic acid monomers; and acrylamide monomers. The following Table 1 is a non-limiting illustration of the polymers and molecular weights possible. (Molecular weights can be determined by an intrinsic viscosity method, such as one using Mark-Houwink-Sakurada constants.)

**Table 1**

| **Polymer Composition** | **Molecular Weight** |
|---|---|
| 99% AMPS 1% VPA | 75,000 |
| | 125,000 |
| | 500,000 |
| | |
| 89% PAM 10% AMPS 1% VPA | 500,000 |
| | 2,000,000 |
| | 5,000,000 |
| | |
| 85% PAM 10% AMPS 5% VPA | 75,000 |
| | 500,000 |
| | 2,000,000 |
| | 5,000,000 |
| AMPS = 2-acrylamido - 2-methylpropanesulfonic acid monomers | |
| VPA = vinylphosphonic acid monomers | |
| PAM = polyacrylamide monomers | |

A non-limiting example of one of the polymers useful in the present invention can be exemplified by the following polymer segment structure:

In a preferred embodiment, the phosphonated substituents are effective for bonding with a mineral filler. Such mineral fillers are those typically used in paper making applications. Non-limiting examples of such fillers are clays, calcium carbonates (such as ground carbonates or precipitated calcium carbonates), and talcs. As will be understood, the phosphonated substituent(s) used and its(their) effectiveness will vary according to the type of paper making materials (e.g. pulps and/or fillers) and manufacturing conditions (e.g. temperatures, pressures, other chemicals) applied. "Bonding" as used herein may include either or both of an acid-base interaction and ionic bonding to create a useful amount of affixation or affinity between the polymer and the mineral filler for the intended utility. Accordingly, bonding can be, but need not be, indicated by secondary measurements, such as retention or strength measurements in paper applications.

In a preferred embodiment, the sulphonated substituents are effective for bonding with a polysaccharide material. Such polysaccharide material can be those typically used in paper making applications, such as starches, fibers, thickening agents and the like. Non-limiting examples of such fiber materials are wood, bamboo, bagasse or other cellulosic biomass. Starch examples are cationic or neutral waxy maize, potato, tapioca, converted or chemically modified starch, synthetic starch, and the like. Thickening agents are the carboxymethyl family of thickeners and the like.

The selection and amount of the optional cationic or neutrally charged amide substituent for reducing the electrostatic charge density and for hydrogen bonding will vary according to the selection of the phosphonated and sulphonated substituents.

The polymeric composition used in this invention can have wide and varying characteristics relating to average molecular weights, molecular weight distributions. charge density, and type of monomeric units. Depending on the application, these characteristics can be adjusted. For instance, in a desired application the average molecular weight might be 1,000,000 with 85% of the polymers having a molecular weight of 1,000,000 ± 15%. As a further example, in another application, 85% of the polymers might have a molecular weight of 1,000,000 ± 50%.

Polymers can be classified as straight polymers and cross-linking polymers. Using known methods of analysis, such as Nuclear Magnetic Resonance Spectrocopy (NMR), the degree of cross-linking polymers (as a weight percent of the total composition) can be ascertained. In a preferred embodiment, the polymer composition has a low degree of cross-linking and contains less than about 15 weight percent; more preferably, less than about 5 weight percent; and even more preferably, less than about 1 weight percent of cross-linking polymers.

In another embodiment of the present invention, instead of the phosphonated substituted having the above-described structure, the composition used in the present invention has in lieu thereof a substituent comprising a derivative of a condensed phosphate, such as of a polyphosphate, pyrophosphate, or polyphosphoric acid (e.g. such as pyrophosphoric acid, metaphosphoric acid, superphosphoric acid or orthophosphoric acid).

In another aspect, an embodiment of the present invention is a method for improving the strength in paper comprising the addition of certain polymers compositions of the above polymer to a paper furnish optionally containing fillers. The preferred polymers are copolymers comprising acrylamide monomers and phosphonated monomers or sulphonated monomers or are terpolymers comprising acrylamide monomers, phosphonated monomers and sulphonated monomers. The addition of the polymer composition can be prior to the headbox of a paper machine in either the thick or thin stock. Split or multiple addition points and other strategies can be used. The amount added will vary according to the nature of the papermaking furnish and the intended use of the paper produced, but should be typically in the range of from about one pound to about five pounds of polymer composition per ton of furnish.

Unexpectedly, the polymer in admixture with starch provides a synergistic increase in the strength of the paper produced. In one aspect, the synergistic effect is signified by the fact that no amount of either additional polymer or starch, when used alone, can provide an equivalent result to the combination of polymer and starch. The starch useable are those typically useable for papermaking. Such starch can be synthetic, such as ethylated or oxidized forms; or organic, such as potato based, preferably cationic potato starch, or corn based, such as cationic waxy maize. When both polymer composition and starch are added to paper furnish, the points of addition for each can be at various points upstream of the headbox. The polymer is preferably added to the thick stock and preferably before the addition of the starch. Split addition of each can be performed. Use of such polymers alone and in combination with starch improves the strength of paper formed with the polymers. Such strength improvement can conveniently be measured using known methods, such as breaking length, mullen burst and Scott bond methods.

Accordingly, one embodiment of the present invention is a process for the production of paper comprising the admixing of starch and a polymer composition comprising one or more polymers of the group consisting of acrylamide polymers, acrylamide polymers co-polymerized with a monomer containing a pendent sulfonic acid group or a phosphonic acid a group, and terpolymers of acrylamide co-polymerized with both a monomer containing a pendant sulfonic acid group and a monomer containing pendant phosphonic acid group. Such admixing occurs prior to or during the preparation of the furnish before providing the furnish to the paper machine. The sequence of the admixing can be before, during or after the addition of the starch and polymer compositions to the furnish, preferably before. When the starch and polymer composition is added to the furnish separately, the preferred order is to add the starch first. The polymer compositions are those described hereinabove.

The preferred process comprises effectively admixing the starch and polymer compositions to produce a paper sheet having a strength unexpectedly significantly greater than when either the starch or polymer composition is used alone, preferably at least about 15% greater, more preferably at least about 50 % greater. Even more preferably at least about 100% greater.

In another aspect, an embodiment of the present invention is a process comprising effectively admixing the starch and polymer composition to produce a paper sheet having an unexpected synergistic increase in strength over the strength when either starch or polymer composition is used alone. Such "Synergistic Increase" is measured by comparing the strength attained by the combination of starch and polymer composition over the absence of both starch and polymer composition in comparison to the additive sums of the separate increases in strength of each of the starch and polymer composition alone over the absence of both starch and polymer compositions in the formed paper. Stated in the form of an equation:

SI = [(SC - SA)/(SA)] - [(SS-SA)/(SA) + (SP-SA)/(SA)] , wherein SI is the synergistic increase, SC is the strength of the paper with the combination of starch and polymer composition, SA is the strength of the paper in the absence of either starch or polymer composition, and SS and SP are the respective strengths of paper with starch and polymer composition alone. The presence of a meaningful value of SI (e.g. that over experimental artifacts) is considered significant and unexpected as indicative of a result better than additive effects. In a preferred embodiment, the synergistic increase is one such that no amount of additional polymer or starch alone when singularly present will provide the equivalent strength provided by the inventive combination of polymer and starch for a given weight percent of inorganic (e.g., filler) material.

The amount of starch useable will vary in accordance with the particular furnish and paper being produced. Such amounts can typically range from about five to about fifty pounds per ton of paper. Similarly, the amount of the polymer composition can typically range from about one to about ten pounds per ton of paper.

The following examples are illustrations of the present invention, but are not intended to be limiting examples inasmuch as other methods are possible.

### EXAMPLE 1

### Preparation of AMPS/PAM/VPA Terpolymer

A flask is charged with 145.0 milliliters of distilled water, 21.75 grams of acrylamide and 4.0 grams of sodium 2-acrylamido-2-methylpropanesulfonic acid monomer (50%) and heated under nitrogen to 70°C. Add approximately 1 gram solid sodium hydroxide to adjust pH to about 7. Then 0.005 grams of potassium persulfate in 5 milliliters distilled water is added and the temperature permitted to rise to 80°C. As mix thickens, add 5 milliliters distilled water. Over a period of about one hour add a feed of 25.0 milliliters distilled water, 11.78 grams of sodium 2-acrylamido-2-methylpropanesulfonic acid monomer (50%), and 0.40 grams of vinylphosphoric acid monomer, together with 2.4 grams of a 10% sodium hydroxide solution to adjust the pH of mix to about 7. As mixture thickens add distilled water (approximately 90 milliliters total over addition period). Fifteen minutes after addition of feed, add 15 milliliters of distilled water. About thirty minutes later, add 0.2 grams of potassium persulfate together with 5 milliliters of distilled water, after 3-4 minutes, add 0.1 grams sodium metabisulfite together with 5 milliliters of distilled water. Maintain the temperature of the mixture remains at about 80°C. Add 200.0 grams of cold distilled water. Continue heating to elevate to 80°C and continue mixing for approximately three hours. Recover. Sample analysis: 5.88% solids; 0.069% residual monomers; 3.4027 intrinsic viscosity (e.g. Mark-Houwink-Sakurada Constants); molecular weight of 999,024.65.

### EXAMPLE 2

### Use Of Polymers in Papermaking

Handsheets were made using a 75% hardwood / 25% softwood blend of bleached northern Kraft pulps, co-refined at 1.6% consistency to an endpoint of 400 Canadian Standard Freeness. The refined pulp was diluted to 0.3125% consistency for papermaking. Hercon 75 cationic alkyl ketene dimer emulsion was added to the furnish at the rate of 0.25%. The terpolymer of the PAM, AMPS and vinylphosphonic acid (VPA) was added to the furnish at the rate of 0.25% when specified. Albacar® HO precipitated calcium carbonate was added to the furnish batch for each set of handsheets in amounts adjusted to achieve filler levels of approximately 14, 21, and 28%. Stalok 400 cationic potato starch was added to the furnish at 0.75% when specified. Reten 1523 anionic polyacrylamide retention aid was added to the furnish at the rate of 0.025%. Each furnish batch was then divided into four aliquots to produce 2.5 gram handsheets (60.6 g/m²). After each handsheet was formed on the Formax (Noble & Wood type) sheet former, it was pressed between a stainless steel roll and a rubber roll at 20 psi, while sandwiched between pieces of paper machine "wet felt" material. These handsheets were dried on a 115°C drum dryer, then conditioned and tested under TAPPI standard conditions of 23°C and 50% relative humidity. The results of the testing are shown in Figures 1 and 2.

### EXAMPLE 3

### Glass Transition Temperatures

Differential scanning calorimetry analysis was performed on five polymer composition sample to determine the presence of singular glass transition temperatures. The results are presented in the following table:

| **Sample No.** | **Molecular Weight** | **AMPS** | **PAM** | **VPA** | **Glass Transition Temperature** |
|---|---|---|---|---|---|
| 1 | 2,100,000 | --- | 100 | --- | 120.9 |
| 2 | 1,800,000 | 10 | 90 | --- | 110.93 |
| 3 | 1,000,000 | --- | 90 | 10 | 78.78 |
| 4 | 500,000 | 10 | 85 | 5 | 83.63 |
| 5 | 1,000,000... | 10 | 89 | 1 | 96.87 °C |
| Molecular weights determined by intrinsic viscosity method. | | | | | |
| AMPS - weight percent 2-acrylamido - 2 - methylpropane sulfonic acid. | | | | | |
| PAM - weight percent polyacrylamide. | | | | | |
| VPA - weight percent vinylphosphonic acid. | | | | | |

## Claims

1. A method for the manufacture of paper comprising adding to a paper furnish a polymer composition comprising a polymeric core; one or more phosphonated substituents and one or more sulphonated substituents; and optionally, one or more cationic or neutrally charged amide substituents.

2. A method according to Claim 1 wherein the polymeric core comprises one or more polymer units selected from alkylic units and vinylic units.

3. A method according to Claim 1 or Claim 2 wherein the phosphonated substituent(s) are of the formula-A-P (=O)(-OD₁)(-OD₂), wherein "P" is phosphorus; "O" is oxygen; and "A" is selected from a carbon-to-phosphorus link or from an unsubstituted or substituted (C₁-C₆) alkylene, wherein the substituent is independently selected from (C₁-C₃) alkyls and halogens, or from a carbonyl (-CO), carbonylaminos, alkylenecarbonylaminos, carbonylaminoalkylenes, or alkylenecarbonylaminoalkylenes; and "D" is a hydrogen proton or a salt moiety selected from aluminum, calcium, iron, lithium, magnesium, potassium, sodium, titanium and zinc ions.

4. The composition of any of the preceding Claims wherein the sulphonated substituent(s) are of the formula -A-S (=O)₂(-OD₁), wherein "S" is sulphur, "O" is oxygen; and "A" is selected from a carbon-to-sulphur link or from an unsubstituted or substituted (C₁-C₆) alkylene, wherein the substituent is independently selected from (C₁-C₃) alkyls and halogens, or from a carbonyl (-CO-), carbonylaminos, alkyllenecarbonylaminos, carbonylaminoalkelenes, or alkylenecarbonylaminoalalkylenes; and "D" is a hydrogen proton or a salt moiety selected from aluminium, calcium, iron, lithium, magnesium, potassium, sodium, titanius and zinc ions.

5. A method according to any of the preceding Claims wherein the cationic or neutrally charged amide substituent is of the formula -A₁-C(=O)-N(B)R₁R₂, wherein "C" is carbon; "O" is oxygen; "N" is nitrogen; "A₁" is an unsubstituted or substituted (C₁-C₆) Ikylene, wherein the substituents are independently selected from (C₁-C₃) alkyls and halogens; and "B" is hydrogen, hydroxyl, or ether; and "R₁" and "R₂" are each independently hydrogen, halogen or a (C₁-C₃) alkyl.

6. A method according to any of the preceding Claims wherein the phosphonated substituent is selected from the group consisting of-PO₃H₂, -PO₃(CH₃)₂, -PO₃(H)(CH₃), -CH₂PO₃H₂, -CH₂PO₃(CH₃) ₂, -CH₂PO₃(H)(CH₃), -C(=O)NHCH₂PO₃H₂; the sulphonated substituent selected from the group consisting of -C(=O)NHC(CH₃)₂CH₂SO₃H, -C(=O)NHCH₂SO₃H, -CH₂C(=O)NHC(CH₃)₂, -CH₂SO₃H, and -CH₂C(=O)N(CH₃)C(CH₃)₂CH₂SO₃H; and the amide substituent selected from the group consisting of -C(=O)NH₂, CH₂C(=O)NH₂-C(=O)NHCH₃, and -C(=O)N⁺(CH₃)₃.

7. A method according to Claim 6 in which the phosphonated substituent is -PO₃H₂; the sulphonated substituent is -C(=O)NHC(CH₃)₂CH₂SO₃H; and the amide substituent is C(=O)NH₂.

8. A method according to any of the preceding Claims wherein the ratio of phosphonated substituents to sulphonated substituents is 10/90 to 1/99.

9. A method according to any of the preceding Claims wherein the ratio of the amide substituent to the phosphonated substituents is 10/1 or higher.

10. A method according to any of the preceding Claims wherein the average molecular weight of the composition ranges from 100,000 to 20,000,000.

11. A method according to any of the preceding Claims wherein there is less than 15 wt % cross-linking.

12. The composition of any of the preceding Claims wherein the cross-linking is less than 1 wt %.

13. A method according to any of the preceding Claims in which the furnish also contains one or more fillers.

14. The method of any preceding Claims further comprising the addition of starch to the paper furnish.

15. The method of Claim 14 wherein the starch is ethylated or oxidised starch or potato based or corn starch.

16. The method of Claim 14 or Claim 15 wherein the amount of starch ranges from five to fifty pounds per ton of paper.

17. The method of any Claims 14 to 16 wherein the amount of the polymer composition ranges from one to ten pounds per ton of paper.

18. A paper composition comprising paper containing fillers and a composition comprising a polymeric core; one or more phosphonated, one ore more sulphonated substituents; and optionally, one or more cationic or neutrally charged amide substituents.

19. A paper composition according to Claim 18 also containing starch.

20. The paper composition of Claim 19 wherein the starch is ethylated or oxidised starch or potato used cornstarch.

## Patentansprüche

1. Verfahren zur Herstellung von Papier beinhaltend die Zugabe zu einem Papierstoff einer Polymerzusammensetzung, welche einen polymeren Kern, einen oder mehr phosphonierte Substituenten und einen oder mehr sulfonierte Substituenten und, optional, einen oder mehr kationische oder neutral geladene Amidsubstituenten enthält.

2. Verfahren nach Anspruch 1, wobei der polymere Kern eine oder mehr polymere Einheiten, die aus Alkyl- und Vinyleinheiten ausgewählt sind, beinhaltet.

3. Verfahren nach Anspruch 1 oder 2, wobei die phosphonierten Substituenten die Formel -A-P(=O)(O-D₁)(O-D₂) besitzen, wobei "P" Phosphor ist, "O" Sauerstoff und "A" aus einer Kohlenstoff-Phosphor-Verbindung oder von einem unsubstituierten oder substituiertem (C₁-C₆)-Alkylen ausgewählt ist, wobei der Substituent unabhängig aus (C₁-C₃)-Alkylen und Halogenen oder aus einer Carbonyl (-CO)-, Carbonylamino-, Alkylencarbonylamino-, Carbonylaminoalkylen- oder Alkylencarbonylaminoalkylengruppe ausgewählt ist; und "D" ein Wasserstoffproton oder ein Salzanteil, ausgewählt aus Aluminium-, Calcium-, Eisen-, Lithium-, Magnesium-, Kalium-, Natrium-, Titan- und Zinkionen ist.

4. Die Zusammensetzung nach einem der vorhergehenden Ansprüche, wobei die sulfonierten Substituenten die Formel -A-S(=O)₂(-OD₁) besitzen, wobei "S" Schwefel ist, "O" Sauerstoff und "A" aus einer Kohlenstoff-Schwefel-Verbindung oder von einem unsubstituerten oder substituiertem (C₁-C₆)-Alkylen ausgewählt ist, wobei der Substituent unabhängig aus (C₁-C₃)-Alkylen und Halogenen oder aus einer Carbonyl (-CO)-, Carbonylamino-, Alkylencarbonylamino-, Carbonylaminoalkylen- oder Alkylencarbonylaminoalkylengruppe ausgewählt ist; und "D" ein Wasserstoffproton oder ein Salzanteil, ausgewählt aus Aluminium-, Calcium-, Eisen-, Lithium-, Magnesium-, Kalium-, Natrium-, Titan- und Zinkionen ist.

5. Verfahren nach einem der vorhergehenden Ansprüche, wobei der kationische oder neutral geladene Amidsubstituent die Formel -A₁-C(=O)-N(B)R₁R₂ besitzt, wobei "C" Kohlenstoff ist, "O" Sauerstoff; "N" Stickstoff" und "A₁" ein unsubstituiertes oder substituiertes (C₁-C₆)-Alkylen, wobei die Substituenten unabhängig aus (C₁-C₃)-Alkylen und Halogenen ausgewählt sind; und "B" Wasserstoff, Hydroxyl oder Ether ist; und "R₁" und "R₂" jeweils unabhängig Wasserstoff, ein Halogen oder ein (C₁-C₃)-Alkyl sind.

6. Verfahren nach einem der vorhergehenden Ansprüche, wobei der phosphonierte Substituent aus einer Gruppe bestehend aus -PO₃H₂, PO₃(CH₃)₂, -PO₃(H)(CH)₃, -CH₂PO₃H₂, CH₂PO₃(CH₃)₂, -CH₂PO₃(H)(CH₃), -C(=O)NHCH₂PO₃H₂ ausgewählt ist, der sulfonierte Substituent aus einer Gruppe bestehend aus -C(=O)NHC(CH₃)₂SO₃H, -C(=O)NHCH₂SO₃H, -CH₂C(=O)NHC(CH₃)₂, -CH₂SO₃H, und -CH₂C(=O)N(CH₃)C(CH₃)₂CH₂SO₃H ausgewählt ist, und der Amidsubstituent aus einer Gruppe bestehend aus -C(=O)NH₂, -CH₂C(=O)NH₂, -C(=O)NHCH₃, und -C(=O)N⁺(CH₃)₃ ausgewählt ist.

7. Verfahren nach Anspruch 6, wobei der phosphonierte Subsituent -PO₃H₂ , der sulfonierte Substituent -C(=O)NHC(CH₃)₂CH₂SO₃H und der Amidsubsituent -C(=O)NH₂ ist.

8. Verfahren nach einem der vorgehenden Ansprüche, wobei das Verhältnis von phosphonierten zu sulfonierten Substituenten von 10/90 bis 1/99 beträgt.

9. Verfahren nach einem der vorhergehenden Ansprüche, bei dem das Verhältnis von Amidsubstituenten zu phosphonierten Substituenten 10/1 oder höher ist.

10. Verfahren nach einem der vorhergehenden Ansprüche, wobei das durchschnittliche Molekulargewicht der Zusammensetzung zwischen 100.000 und 20.000.000 beträgt.

11. Verfahren nach eine der vorhergehenden Ansprüche, wobei der Grad an Quervernetzung weniger als 15% Gewichtsprozent beträgt.

12. Verfahren nach eine der vorhergehenden Ansprüche, wobei der Grad an Quervernetzung weniger als 1% Gewichtsprozent beträgt.

13. Verfahren nach einem der vorhergehenden Ansprüche, wobei der Eintrag noch einen oder mehrere Füllstoffe enthält.

14. Verfahren nach einem der vorhergehenden Ansprüche, weiterhin beinhaltend die Zugabe von Stärke zu dem Papierstoff.

15. Verfahren nach Anspruch 14, wobei die Stärke ethylierte oder oxidierte Stärke oder Kartoffel- oder Maisbasierte Stärke ist.

16. Verfahren nach Anspruch 14 oder 15, wobei die Menge an Stärke im Bereich von 5 bis 50 Pfund pro Tonne Papier liegt.

17. Verfahren nach einem der Ansprüche 14 bis 16, wobei die Menge an Polymerzusammensetzung im Bereich von einem bis 10 Pfund pro Tonne Papier beträgt.

18. Eine Papierzusammensetzung beinhaltend Papier, welches Füllstoffe und eine Zusammensetzung mit einem polymeren Kern, einem oder mehr phosphonierten, einem oder mehr sulfonierten und optional einem oder mehr kationisch oder neutral geladenen Amidsubstituenten beinhaltet.

19. Eine Papierzusammensetzung nach Anspruch 18, welche zusätzlich Stärke enthält.

20. Die Papierzusammensetzung nach Anspruch 19, wobei die Stärke ethyliert oder oxidiert ist oder Kartoffelbenutzte Maisstärke ist.

## Revendications

1. Procédé pour la production de papier, comprenant l'addition à une composition de fabrication de papier d'une composition polymère comprenant une partie centrale polymère ; un ou plusieurs substituants phosphonés et un ou plusieurs substituants sulfonés ; et, facultativement, un ou plusieurs substituants amide cationiques ou de charge neutre.

2. Procédé suivant la revendication 1, dans lequel la partie centrale polymère comprend un ou plusieurs motifs polymères choisis entre des motifs alkyliques et des motifs vinyliques.

3. Procédé suivant la revendication 1 ou la revendication 2, dans lequel le ou les substituants phosphonés répondent à la formule -A-P(=O)(-OD₁)(-OD₂), dans laquelle "P" représente un atome de phosphore ; "O" représente un atome d'oxygène ; et "A" est choisi entre une liaison carbone-phosphore et un groupe alkylène en C₁ à C₆ non substitué ou substitué, dans lequel le substituant est choisi, indépendamment, entre des substituants alkyle en C₁ à C₃ et halogéno, ou entre des substituants carbonyle (-CO), carbonylamino, alkylènecarbonylamino, carbonylaminoalkylène et alkylènecarbonylamino-alkylène ; et "D" représente un proton d'hydrogène ou un groupement de sel choisi parmi les ions aluminium, calcium, fer, lithium, magnésium, potassium, sodium, titane et zinc.

4. Composition suivant l'une quelconque des revendications précédentes, dans laquelle le ou les substituants sulfonés répondent à la formule -A-S(=O)₂(-OD₁), dans laquelle "S" représente un atome de soufre, "O" représente un atome d'oxygène et "A" est choisi entre une liaison carbone-soufre et un groupe alkylène en C₁ à C₆ non substitué ou substitué, dans lequel le substituant est choisi, indépendamment, entre des substituants alkyle en C₁ à C₃ et halogéno, ou entre des groupes carbonyle (-CO-), carbonylamino, alkylènecarbonylamino, carbonylaminoalkylène et alkylènecarbonylamino-alkylène ; et "D" représente un proton d'hydrogène ou un groupement de sel choisi parmi les ions aluminium, calcium, fer, lithium, magnésium, potassium, sodium, titane et zinc.

5. Procédé suivant l'une quelconque des revendications précédentes, dans lequel le substituant amide cartionique ou de charge neutre répond à la formule -A₁-C(=O)-N(B)R₁R₂, dans laquelle "C" représente un atome de carbone, "O" représente un atome d'oxygène, "N" représente un atome d'azote, "A₁" représente un groupe alkylène en C₁ à C₆ non substitué ou substitué, dans lequel les substituants sont choisis, indépendamment, entre des substituants alkyle en C₁ à C₃ et halogéno ; et "B" représente un atome d'hydrogène, un groupe hydroxyle ou un groupe éther ; et "R₁" et "R₂" représentent chacun, indépendamment, un atome d'hydrogène, un atome d'halogène ou un groupe alkyle en C₁ à C₃.

6. Procédé suivant l'une quelconque des revendications précédentes, dans lequel le substituant phosphoné est choisi dans le groupe consistant en des substituants -PO₃H₂, -PO₃(CH₃)₂, -PO₃(H)(CH₃), -CH₂PO₃H₂, -CH₂PO₃(CH₃)₂, -CH₂PO₃(H)(CH₃) et -C(=O)NHCH₂PO₃H₂ ; le substituant sulfoné est choisi dans le groupe consistant en des substituants -C(=O)NHC(CH₃)₂CH₂SO₃H, -C(=O)NHCH₂SO₃H, -CH₂C(=O)NHC(CH₃)₂, -CH₂SO₃H et -CH₂C(=O)N(CH₃)C(CH₃)₂CH₂SO₃H ; et le substituant amide est choisi dans le groupe consistant en des substituants -C(=O)NH₂, CH₂C(=O)NH₂C(=O)NHCH₃ et -C(=O)N⁺(CH₃)₃.

7. Procédé suivant la revendication 6, dans lequel le substituant phosphoné est un substituant -PO₃H₂ ; le substituant sulfoné est un substituant -C(=O)NHC(CH₃)₂CH₂SO₃H et le substituant amide est un substituant C(=O)NH₂.

8. Procédé suivant l'une quelconque des revendications précédentes, dans lequel le rapport des substituants phosphonés aux substituants sulfonés est compris dans l'intervalle de 10/90 à 1/99.

9. Procédé suivant l'une quelconque des revendications précédentes, dans lequel le rapport du substituant amide aux substituants phosphonés est égal ou supérieur à 10/1.

10. Procédé suivant l'une quelconque des revendications précédentes, dans lequel le poids moléculaire moyen de la composition est compris dans l'intervalle de 100 000 à 20 000 000.

11. Procédé suivant l'une quelconque des revendications précédentes, dans lequel il existe moins de 15 % en poids de réticulation.

12. Composition suivant l'une quelconque des revendications précédentes, dans laquelle le taux de réticulation est inférieur à 1 % en poids.

13. Procédé suivant l'une quelconque des revendications précédentes, dans lequel la composition de fabrication contient également une ou plusieurs charges.

14. Procédé suivant l'une quelconque des revendications précédentes, comprenant en outre l'addition d'amidon à la composition de fabrication de papier.

15. Procédé suivant la revendication 14, dans lequel l'amidon est un amidon éthylé ou oxydé ou un amidon dérivé de la pomme de terre ou bien l'amidon de mais.

16. Procédé suivant la revendication 14 ou la revendication 15, dans lequel la quantité d'amidon est comprise dans l'intervalle de cinq à cinquante livres par tonne de papier.

17. Procédé suivant l'une quelconque des revendications 14 à 16, dans lequel la quantité de composition polymère est comprise dans l'intervalle d'un à dix livres par tonne de papier.

18. Composition de papier, comprenant du papier contenant des charges et une composition comprenant une partie centrale polymère ; un ou plusieurs substituants phosphonés, un ou plusieurs substituants sulfonés ; et, facultativement, un ou plusieurs substituants amide cationiques ou de charge neutre.

19. Composition de papier suivant la revendication 18, contenant également de l'amidon.

20. Composition de papier suivant la revendication 19, dans laquelle l'amidon est un amidon éthylé ou oxydé ou un amidon dérivé de la pomme de terre ou bien l'amidon de maïs.
